

# United States Patent

Carpenter et al.

[15] 3,700,762

[45] Oct. 24, 1972

[54] PROPELLANT GRAIN

[72] Inventors: David W. Carpenter; Charley R. Rodgers, both of China Lake, Calif.

[73] Assignee: The United States of America as represented by the Secretary of the Navy

[22] Filed: May 4, 1970

[21] Appl. No.: 34,032

[52] U.S. Cl. ....264/3, 102/103, 149/5

[51] Int. Cl. ....C06b 21/02

[58] Field of Search .....102/103; 264/3; 149/5, 6, 7

[56] References Cited

## UNITED STATES PATENTS

3,202,557 8/1965 Kaufman .....102/103

|           |         |                                |
|-----------|---------|--------------------------------|
| 3,426,528 | 2/1969  | Mangum et al.....102/103       |
| 3,493,446 | 2/1970  | Braum.....102/103              |
| 3,108,433 | 10/1963 | De Fries et al. ....102/103    |
| 2,958,288 | 11/1960 | Campbell, Jr. et al....102/103 |
| 2,995,011 | 8/1961  | Kimmel.....264/3               |
| 3,144,830 | 8/1964  | De Fries et al. ....102/103    |

Primary Examiner—Benjamin A. Borchelt

Assistant Examiner—H. J. Tudor

Attorney—R. S. Sciascia, Roy Miller and Gerald F. Baker

[57]

## ABSTRACT

A propellant grain is wrapped with glass fiber tape and fitted with epoxy end pieces to inhibit burning in those areas. A fluorocarbon grain is etched with hydrochloric acid and then immersed in lacquer before being wrapped.

2 Claims, 3 Drawing Figures



PATENTED OCT 24 1972

3,700,762



FIG. 2.



FIG. 3.

INVENTORS.  
DAVID W. CARPENTER  
CHARLEY R. RODGERS  
BY ROY MILLER  
ATTORNEY.  
GERALD F. BAKER  
AGENT.

## PROPELLANT GRAIN

## BACKGROUND OF THE INVENTION

Because previous inhibiting methods for cartridge loaded propellant grains were found to be impractical for fluorocarbon propellant grains, new methods and materials for providing inhibitors were necessarily developed. The old inhibitor materials such as ethyl cellulose and cellulose acetate were found to be inapplicable to fluorocarbon grains because such materials will not bond to the binders used in these grains. The inhibitor means provided by the present invention provides thermal protection to the motor tube and eliminates need for heat barriers and also reduces overall motor costs. The peripheral inhibitor tape further provides structural integrity to the grain under high centrifugal loading.

## BRIEF DESCRIPTION OF THE SEVERAL VIEWS OF THE DRAWING:

FIG. 1 is a side view partly in longitudinal cross section of a propellant grain provided with inhibitors according to the present invention;

FIG. 2 is an end view of the grain in FIG. 1; and

FIG. 3 is a detail view.

## DETAILED DESCRIPTION OF THE INVENTION:

As shown in FIG. 1, a propellant grain 10 is fitted with two end inhibitors 12, 14 of epoxy resin or the like the grain is wrapped with inhibiting tape 16. The propellant grain 10 is typical and is shown with a bore 13 and, one end, a counterbore 20. The other end has an inner tapered portion 22.

Looking at FIG. 2 we see that the illustrated propellant grain is formed with a number of convolutions 17. The number and configuration of convolutions varies with size and design. The simplest design, for example, comprises two orthogonal longitudinal passages.

The fragmentary view in FIG. 3 shows the propellant

40

grain 10 with two wrappings of inhibiting tape 16 and shows the manner of laying up the inhibiting tape with a typical lap joint, for example, of 1 1/16 inches.

The propellant grains may be formed by any known process but typically are cast in molds. The grain as it comes from the mold is prepared by covering the ends with tape and then cleansing the remaining surface with soap and cold water. The grain is then dried with a clean wiper, immersed in a 1:1 solution of HCl and etched for 45 minutes.

The etched grains are then rinsed in cool running water, wiped dry and the tape is removed from the ends after which the grains are vacuum dried in an oven at 135° F. A ring of flexible epoxy is next cast in situ on each end of the grain and after each ring is cast the grain is placed in an oven at 180° - 200° F. for at least 1 1/4 hours to cure the epoxy.

Internal casting fixtures are used in casting the end pieces and these fixtures are left in place for the next 20 operation which consists of three immersions in Viton lacquer interspersed with half hour drying periods.

Finally the outer surface of the grain is wrapped with tape. The tape is preferably applied using a tape wrapping lathe and is applied in two or more layers. A 25 tape found suitable for this application is a 2-inch wide tape manufactured by Minnesota Mining and Manufacturing Company and designated as Y 9087.

What is claimed is:

1. The process of manufacture of a propellant grain including the steps of:

30 molding propellant material into a hollow solid having inner and outer substantially cylindrical surfaces;

chemically treating said outer surfaces by bathing in a 1:1 solution of HCL;

coating said outer surfaces with lacquer; and

wrapping said outer surfaces with glass fiber tape.

2. The process of claim 1 wherein said propellant material comprises a fluorocarbon.

\* \* \* \* \*

45

50

55

60

65